

## UNITED STATES PATENT OFFICE

2,304,884

## COLOR PHOTOGRAPHY

Burt H. Carroll, Rochester, N. Y., assignor to  
Eastman Kodak Company, Rochester, N. Y., a  
corporation of New Jersey

No Drawing. Application April 8, 1941, Serial No.  
387,450. In Great Britain April 9, 1940

10 Claims. (Cl. 95—6)

This invention relates to color photography and particularly to an improved material for the bleach-out method of color photography.

Processes of color photography are known which make use of uniformly dyed silver halide emulsions, the colored image being formed by destroying the dye in the regions of a silver or silver salt image. The dye incorporated in the gelatin or emulsion may possess a color which is complementary to that of the light which the sensitive emulsion is intended to record or may be such as to transmit it freely.

This invention relates to processes of the former type in which the dye incorporated in the gelatin or emulsion is complementary in color to that of the light which the emulsion is intended to record. In such processes the dye which is used has its light absorption maximum at a wave length which is substantially identical with the maximum sensitivity of the emulsion in which the dye is incorporated. There is, therefore, a loss in sensitivity because the maximum absorption of the dye corresponds to the region of maximum sensitivity of the emulsion. This inherent limitation on speed, combined with desensitizing action of the coloring dyes, which is usually found in practice, limits the process to use with printing materials and requires relatively sensitive emulsions in order to secure a working sensitivity adequate for enlarging.

It is, therefore, an object of the present invention to provide a material which retains the inherent advantage of this type of bleach-out process, affording direct color positives, while increasing the speed of the material. Another object is to provide a novel method of coloring emulsion layers for the bleach-out process of color photography. A still further object is to provide a method of increasing the effective sensitivity of silver halide emulsion layers used in the bleach-out process of color photography. Other objects will appear from the following description of my invention.

These objects are accomplished by treating dyes suitable for use in the bleach-out method of color photography so that their absorption maxima are shifted from the region of maximum sensitivity of the layers in which they are incorporated, and after exposure, reconverting the dyes to dyes having the proper colors for image dyes. This is accomplished by forming in the photographic layer a dye derivative by treatment of a dye with a metallic salt, preferably an alkaline earth metal salt of an inorganic acid, prior to exposure and subsequently restoring the dye to a form having the

proper light absorption and transmission characteristics for an image forming dye.

When the dyes used in the photographic layers are treated with metallic salts according to the present invention, the metallic derivatives so formed have a color which differs from that of the original dye by an amount sufficient to cause an appreciable reduction in the light absorption of the dye in the region which the emulsion is intended to record and, therefore, an increase in the effective sensitivity of the layer is obtained. The change in the light absorption of the dye need not be excessive. For example, a change in the absorption maximum of a blue-green dye from 630 millimicrons to 600 millimicrons has been found to increase the effective speed of the layer in which it is incorporated six times or more. Any suitable dyes which give a metallic derivative, preferably an insoluble derivative, on treatment with a metallic salt may be used, especially polyazo acid dyes.

The metallic salts are preferably alkaline earth salts such as barium, magnesium, or strontium salts, but other heavy metal salts may be used, such as cobalt or nickel salts or salts of complex cations containing metals. Generally, those metallic salts are preferred which change the light absorption maximum of the dye to a shorter wave length since most absorption bands fall off more sharply on the long wave length side of the maximum.

After exposure of the dyed layer to form an image in the layer, the dye is converted to another form, preferably to its original form, by suitable treatment whereby the metal of the added metallic salt is either removed from the dye as a soluble derivative or precipitated in the layer by double decomposition of the dye derivative. Some metals may be partially or wholly removed from the dye during development of the layer in the form of their carbonate or sulfites which may be slightly soluble, but it is generally necessary to take special steps to insure that the whole of the metal is removed from the layer or suitably precipitated in the layer. For example, the metal may be fully removed from the layer during bleaching of the dye by using strong acid baths and subjecting the layer to prolonged washing or

the metal may be removed from the dye by precipitation within the layer, by treatment with a bath containing a soluble salt such as a sulfate, which forms an insoluble compound of the metal, preferably a colorless compound. If desired, such a bath may be incorporated with one or more of

the baths used for processing the layer to a colored image.

The proposed method may be applied to multi-color photographic processes, for example, a three-color process, using photographic elements comprising a plurality of differentially color-sensitive layers coated on a single support. In a three-color process, for example, a sensitive element may comprise a gelatino silver halide emulsion sensitized to red light and dyed uni-

5  
10

The following dyes are specifically suitable for use according to my invention:

The following blue-green dyes

Pontamine Fast Green 5BL

Solophenyl Fast Blue-Green BL

(The dyes of this type are described in Richard U. S. Patent 1,829,673, granted October 27, 1931.) They are believed to have the following formula or substantially similar constitutions:



formly with a blue-green, a gelatino-silver halide emulsion sensitive to green light and dyed uniformly with a magenta dye, and a not-especially color-sensitized gelatino-silver halide emulsion layer dyed uniformly with a yellow dye. One or more of three image-forming dyes should be such that they form metallic salts of a different shade when treated with suitable metallic salts. Preferably the difference in the absorption maximum of the dye and its metallic salt should be at least 20 millimicrons and preferably from 30 to 50 millimicrons. After exposure of the element to 20  
30  
35  
40  
45  
50  
55  
60  
65  
70  
75

form an image or images, a silver image or images are produced in the layers by primary or reversal development and a colored image or images formed by decolorizing or destroying one or more of the dyes in accordance with well known methods such as those described in Christensen U. S. Patent 1,517,049, granted November 25, 1924, and Seymour U. S. Patent 2,184,022 granted December 19, 1939. After formation of the colored image or images, the remaining silver and silver halide in the layers may be removed in any suitable manner.

The dyes may be restored to their original form and shade at any convenient stage in the processing provided that they remain in their converted and shifted absorption form during exposure.

Dyes which I may use include blue to blue-green dyes having the following groupings present in their molecules:



or



where

R=arylamine  
aryl radical containing an azo group  
—N=N—aryl

R<sub>1</sub>=H, alkyl, alkoxy

R<sub>2</sub>=either hydrogens or a fused benzene ring  
(forming naphthalene).

The dyes must also contain one or more salt-forming groups, such as sulfonic acid groups, and may contain other substituent groups.

The dyes having the following formulas:



(This dye is obtained by diazotizing metanilic acid and coupling in acid medium with 1-naphthylamine-6-sulfonic acid, diazotizing the resulting dye and coupling in acid medium with 2-ethoxy-1-naphthylamine-6-sulfonic acid, diazotizing the resulting dye and coupling in alkaline medium with 2-amino-5-naphthol-7-sulfonic acid. The finished dye as the sodium salt corresponds to the above structural formula.)



60

Numbers in the first column are those given to these dyes in Schultz-Lehmann, Farbstofftabellen 7th edition.





(This dye is prepared by diazotizing 1 mole of 1-amino-8-naphthol-3,6-disulfonic acid and coupling it in acid medium with 1 mole of a-naphthylamine, again diazotizing and coupling in alkaline medium with 1 mole of 1-amino-8-naphthol-3,6-disulfonic acid.)

The absorption maxima of the above dyes may be shifted toward the shorter wave length by converting the dyes to their barium salts. They may be used to color the red sensitive layer of a multi-layer element.

Benzo Light Yellow RL (Schultz Lehmann Farbstofftabellen, 7th edition, No. 307). This dye is believed to have the following structural formula:



The above dye may be converted to a form having its absorption maximum shifted toward shorter wave lengths by treatment with cobalt hexamino nitrate to form a cobalt complex salt.

My invention may be further illustrated by the following specific examples:

*Example 1*

To a red-sensitized emulsion dyed with Pontamine Fast Green 5BL or Solophenyl Fast Blue-Green BL there is added a water-soluble barium salt such as barium nitrate or barium acetate in an amount of the order of the weight of the dye, that is, an amount in excess of that necessary to combine with the dye. Since the dye exists as its sodium salt an excess of barium salt is necessary in order to displace the sodium ions by mass action, the barium salts of the dye being slightly soluble. The dye is thus changed from a blue-green dye with an absorption maxima at about 630 millimicrons to a blue dye with an absorption maxima of about 600 millimicrons and the sensitivity of the layer is several times greater than that of the layer dyed with the sodium salt form of the dye.

On exposure and processing the layer, the barium is first removed as carbonate or sulfite during development. The dye then reverts to its original color. During bleaching of the layer, the barium will be permanently removed if

strongly acid bleach baths and long washing times are used.

*Example 2*

To an unsensitized gelatin silver halide emulsion dyed with Benzo Light Yellow RL (Schultz No. 307) there is added an excess of cobalt hexamino nitrate. The dye becomes nearly colorless by formation of the corresponding salt. On exposure and processing of the layer, the original color of the dye is restored by elimination of the cobalt complex.

I realize that some of the dyes used as examples in the present specification have previously been described for use in photographic emulsion layers. However, I claim as novel the discovery that the absorption maxima of these dyes may be shifted to a region outside the region of maximum sensitivity of an emulsion layer in which they are to be incorporated and the effective sensitivity of the layer thereby increased.

I claim:

1. A light-sensitive silver halide layer for the bleach-out process of color photography, effectively sensitive to only one of the primary colors, said layer being uniformly colored with a salt of a polyazo dye selected from the group consisting of alkaline earth metal salts, nickel, and cobalt, the sodium salt of said dye having an absorption maximum at substantially the sensitivity maximum of the layer, but the first mentioned salt having a light absorption maximum at a substantially lower wave length than the sensitivity maximum of said layer, said first-mentioned salt of said dye being convertible into a form having an absorption maximum at substantially the sensitivity maximum of the layer.

2. A light-sensitive silver halide layer for the bleach-out process of color photography, effectively sensitive to only one of the primary colors, said layer being uniformly colored with an alkaline earth metal salt of a polyazo dye, the sodium salt of said dye having an absorption maximum at substantially the sensitivity maximum of the layer, but the alkaline earth metal salt having a light absorption maximum at a substantially lower wave length than the sensitivity maximum of said layer, said alkaline earth metal salt of said dye being convertible into a form having an absorption maximum at substantially the sensitivity maximum of the layer.

3. A gelatin silver halide for the bleach-out process of color photography effectively sensitive to only the red spectral region said layer being uniformly colored with an alkaline earth metal salt of a polyazo dye, the sodium salt of said dye having an absorption maximum at substantially the sensitivity maximum of the layer, but the alkaline earth metal salt having a light absorption maximum at a substantially lower wave length than the sensitivity maximum of said layer, said alkaline earth metal salt of said dye being convertible into a form having an absorption maximum at substantially the sensitivity maximum of the layer.

4. A light-sensitive silver halide layer for the bleach-out process of color photography effectively sensitive to only one of the primary colors, said layer being uniformly colored with a barium salt of a polyazo dye, the sodium salt of said dye having an absorption maximum at substantially the sensitivity maximum of the layer but the barium salt having a light absorption maximum at a substantially lower wave length, and

said barium salt of said dye being convertible after exposure of the layer, to a form having an absorption maximum at substantially the sensitivity maximum of the layer.

5. A light-sensitive gelatino-silver halide layer for the bleach-out process of color photography colored with the barium salt of a dye having the following formula:



where  $X$ =hydrogen, amino hydroxyl,  $Y$ =hydrogen, methyl, methoxy, and from 1 to 2  $Z$ 's of each naphthyl radical are the barium salt of sulfonic acid, the remaining  $Z$ 's being hydrogen, said barium salt having a light absorption maximum not corresponding to the sensitivity maximum of the silver halide layer, but the sodium salt of the dye having a light absorption maximum at substantially the sensitivity maximum of the layer.

6. A light-sensitive gelatino-silver halide layer for the bleach-out process of color photography colored with the barium salt of a dye having the following formula:



where  $Y$ =hydrogen, methyl, methoxy; and from 1 to 2  $Z$ 's of each naphthyl radical are the barium salt of sulfonic acid, the remaining  $Z$ 's being hydrogen, said barium salt having a light absorption maximum not corresponding to the sensitivity maximum of the silver halide layer, but the sodium salt of the dye having a light absorption maximum at substantially the sensitivity maximum of the layer.

7. A light-sensitive gelatino-silver halide layer for the bleach-out process of color photography uniformly colored with the barium salt of Pontamine Fast Green 5BL, said barium salt having a light absorption maximum not corresponding to the sensitivity maximum of the silver halide layer, but the sodium salt of the dye having a light absorption maximum at substantially the sensitivity maximum of the layer.

8. A light-sensitive gelatino-silver halide layer for the bleach-out process of color photography

uniformly colored with a cobalt complex salt of the dye having the following structural formula



10

said cobalt salt having a light absorption maximum not corresponding to the sensitivity maximum of the silver halide layer, but the sodium salt of the dye having a light absorption maximum at substantially the sensitivity maximum of the layer.

9. The method of increasing the effective sensitivity of a silver halide photographic layer used in the bleach-out process of color photography, which comprises converting an azo dye having a light absorption maximum in the region which said layer records, into a salt of said dye selected from the group consisting of alkaline earth metal salts, nickel and cobalt, the sodium salt of said dye having an absorption maximum at substantially the sensitivity maximum of the layer but said first mentioned salt having a light absorption maximum in a region of substantially lower wave-length and incorporating said salt in said emulsion layer.

10. A light-sensitive silver halide layer for the silver bleach-out process of color photography colored with the barium salt of a dye selected from the group consisting of dyes having the following structure:



40

45

50

55

55

60

where  $R$  is selected from the class consisting of hydrogen, alkyl, and alkoxy groups;  $X$  is selected from the class consisting of hydrogen, amino, and hydroxyl groups;  $Y$  is selected from the class consisting of arylamino and azo groups; and the naphthol nucleus contains at least one sulfonic acid radical capable of forming said barium salt, said barium salt having a light-absorption maximum not corresponding to the sensitivity maximum of the silver halide layer, but the sodium salt of the dye having a light-absorption maximum at substantially the sensitivity maximum of the layer.

BURT H. CARROLL.